

May 27, 1958

A. M. BOUNDS ET AL

2,836,491

TUNGSTEN-TITANIUM-NICKEL CATHODES

Filed June 17, 1957

4 Sheets-Sheet 1



May 27, 1958

A. M. BOUNDS ET AL

2,836,491

TUNGSTEN-TITANIUM-NICKEL CATHODES

Filed June 17, 1957

4 Sheets-Sheet 2

Fig. 2A



Fig. 2B



May 27, 1958

A. M. BOUNDS ET AL.

2,836,491

TUNGSTEN-TITANIUM-NICKEL CATHODES

Filed June 17, 1957

4 Sheets-Sheet 3

Fig. 3A



Fig. 3B



May 27, 1958

A. M. BOUNDS ET AL

2,836,491

TUNGSTEN-TITANIUM-NICKEL CATHODES

Filed June 17, 1957

4 Sheets-Sheet 4

*Fig. 4A*



*Fig. 4B*



# United States Patent Office

2,836,491

Patented May 27, 1958

1

2,836,491

## TUNGSTEN-TITANIUM-NICKEL CATHODES

Ardrey M. Bounds, Laverock, and Richard L. Hoff, Norristown, Pa., assignors to Superior Tube Company, Norristown, Pa., a corporation of Pennsylvania

Application June 17, 1957, Serial No. 666,053

4 Claims. (Cl. 75—170)

This invention relates to electron tube cathodes of the indirectly-heated type.

In general, the object of the invention is to provide indirectly-heated cathodes which have, as compared to prior nickel alloy cathodes, substantially enhanced resistance to deformation at cathode-operating temperatures and which have emission and sublimation characteristics substantially equivalent to or better than those of prior nickel or nickel alloy cathodes.

In accordance with the present invention, such objective is attained by making the cathode sleeves or the like from nickel cathode alloys which include the additives tungsten and titanium within the low and narrow limits hereinafter specified.

In the following description, reference is made to the accompanying drawings in which:

Fig. 1 is a group of curves exemplary of the yield strength, at cathode-operating temperatures, of various tungsten-titanium-nickel alloys and of a reference-nickel cathode alloy; and

Figs. 2A, 2B, 3A, 3B and 4A, 4B comprise groups of curves referred to in discussion of the emission characteristics of indirectly-heated cathodes of the reference-nickel alloy and of tungsten-titanium-nickel alloys.

In general, indirectly-heated cathodes consist of a nickel alloy base element, such as a sleeve or cup, having thereon a coating of alkaline earth metals, such as barium, strontium or the like. The fabrication of the alloy stock into the cathode base elements involves hot and cold working steps, such as forging, rolling, drawing, stamping and the like. After assembly of the coated cathode, including its heater and other electrodes within an envelope to form an electronic tube, the cathode is activated by temporarily heating it substantially above its normal operating temperature. During activation, reactions between the base element materials and the coating materials convert the coating into a combination of complex oxides suited to emit electrons when heated to cathode-operating temperatures. In the more usual types of service, the life of a tube is considered terminated when its cathode emission is definitely subnormal at normal heater current. For many uses, including field service where the available supply voltage may be low or fluctuating, tubes are considered unfit for use when the cathode emission is substantially affected by low or varying heater temperature.

The operating life of a tube is also affected by cathode characteristics other than electron emission. Eruptive flaking or peeling of its cathode coating shortens the normal life of tubes, particularly high-voltage rectifier tubes. The formation and growth of a high-impedance interface between the cathode base element and its oxide coating adversely affects tube operation. The resistive component of such interface is damaging, particularly in pulse type service, and even at ordinary frequencies: the capacitive component of such interface impedance is particularly damaging at high frequencies—even when the tube is not operated under pulsed or cut-off condi-

2

tions. The operating life of a tube may also be effectively terminated by the formation, from material sublimed from the cathode, of a leakage path between electrodes of the tube. In addition to such electrical characteristics, the operating life of a tube is also determined by the physical or mechanical characteristics of its cathode. Cathode sleeves made of the usual nickel alloys often bowed when subjected to high activation temperatures, causing internal short-circuits or change in interelectrode spacing. Also in services where the tubes were subjected to severe mechanical shock, as in airborne missile equipment, buckling or deformation of their cathode sleeves rendered the tubes inoperative before performance of their intended function.

We have determined that the addition of tungsten and titanium within the narrow percentage ranges later herein specified, to nickel cathode alloys, provides indirectly-heated cathodes, which have, at cathode-operating temperatures, a hot strength at least several times that of nickel-cathode alloys and which have a high level of stable emission equal to or better than that of nickel cathodes. Furthermore, such tungsten titanium-nickel alloys are amenable to hot and cold metal working steps incident to fabrication of cathode sleeves and the like from the alloy stock. Such cathodes also exhibit the characteristics of virtual freedom from sublimation and of negligible interface impedance.

Considering first the enhancement of yield strength at cathode-operating temperatures of about 1600° F., it is known that the addition of tungsten alone effects an increase in hot strength. Such increase is substantially proportional to the percentage of tungsten added. Increasing the percentage of tungsten from 2% to 4%, for example, increases the hot strength of a nickel-cathode alloy from about 3800 p. s. i. (pounds per square inch) to 4800 p. s. i. as compared to a value of 2500 p. s. i. for the reference-nickel alloy. It is not considered practical however, to increase the amount of tungsten much above 4% because of cathode fabrication difficulties. On the other hand, we have found that the hot strength of such a tungsten-nickel alloy may be further substantially increased without encountering fabrication difficulties by the addition of titanium. Specifically, the addition of 0.15% titanium to a 4% tungsten-nickel alloy increases the hot yield strength to 6250 p. s. i. and the addition of 0.4% titanium to the tungsten-nickel base alloy increases the yield strength to 7650 p. s. i. However, the addition of 2.6% titanium to the tungsten-nickel base increases the hot yield strength to only 7450 p. s. i., indicating that the increase in hot strength is not proportional to the addition of titanium. The strength of a tungsten-titanium-nickel alloy, containing titanium in the range of 0.05% to 3%, at cathode-operating temperatures, is about twice that of the 4% tungsten-nickel alloy and over three times the hot strength of the nickel base alloy.

From tests on binary titanium-nickel cathode alloys, it was determined that addition of titanium to nickel increases the activation so rapidly with increase of titanium that a cathode having only .5% titanium activates quickly to extremely high levels, but quickly deteriorates to unsatisfactory low levels. However, in combination with tungsten as an additive to nickel, the effect of the addition of titanium in the range of 0.05% to 3% is both substantially to increase the hot strength and to provide good emission characteristics throughout a long cathode-operating life. In short, tungsten and titanium interact favorably with regard both to the mechanical and the electrical properties of indirectly-heated cathodes.

From metallographic investigation, it appears that the addition of tungsten and titanium produces precipitation hardening at temperatures below 1200° F. However, at

cathode-operating temperatures of 1600° F. or higher, this second phase is dissolved into the solid solution. For this reason, the marked enhancement of hot strength resulting from small additions of titanium to the tungsten-nickel alloy is attributed to the mechanism of solid solution hardening resulting from the additional presence of titanium.

Data compiled on the emission characteristics of indirectly-heated cathodes made of nickel alloys, tungsten-nickel alloys, titanium-nickel alloys and tungsten-titanium-nickel alloys indicates interaction of the tungsten and titanium in enhancement of, or maintenance of, the emission characteristics of nickel cathodes as well as a substantial increase in their resistance to deformation when subjected to severe mechanical shock while at cathode-operating temperatures. Such effects were not predictable from knowledge of the prior art.

For nickel-cathode alloys containing from about 1% to about 5% tungsten by weight, titanium may be added in the range of from about 0.05% to 3%. Except for residuals and one or more activating agents, the balance of the alloy is essentially the nickel base usually including cobalt not in excess of 1%. Inclusion of higher percentages of cobalt, even up to 10% or 15%, has been found to have little effect upon the emission characteristics or upon the mechanical strength at cathode-operating temperatures.

In these tungsten-titanium-nickel cathode alloys, magnesium and/or aluminum may be used in small controlled quantities as additional activating agents. The percentage of magnesium should not be much in excess of 0.07% to insure a low rate of sublimation. The percentage of aluminum should not be much in excess of 0.15% to avoid peeling of the oxide coating. Because of its effect upon interface impedance, use of silicon as an activating agent should be avoided; if present, the concentration of silicon should not exceed 0.05%.

In determination of the limits of tungsten and titanium for obtaining both enhanced hot strength of indirectly-heated cathodes and preservation or enhancement of emission properties, tests were conducted on a number of tungsten-titanium-nickel cathode alloys. Specific examples of such alloys are listed below in Table A.

Table A

| Alloy  | Ti   | W    | Al   | Mg   | Si   | Fe   | Mn   | C    | Cu   | Co   | Ni                       |
|--------|------|------|------|------|------|------|------|------|------|------|--------------------------|
| #552   | .153 | 3.04 | .132 | .057 | .015 | .020 | .009 | .114 | .013 | 4.72 |                          |
| #5514  | .421 | 4.05 | .127 | .060 | .013 | .025 | .048 | .113 | .009 | 4.64 |                          |
| #54027 | 2.72 | 4.67 | .112 | .037 | .015 | .105 | .130 | .10  |      | .052 | Essentially<br>Remainder |
| #54053 | 2.64 | 3.37 | .140 | .06  | .018 | .125 | .105 | .085 | .013 | .127 |                          |
| 220*   | 0    | 0    | .008 | .035 | .024 | .067 | .128 | .061 | .022 | .540 |                          |
| A31**  | .003 | 3.93 | .004 | .025 | .014 | .032 | .05  | .04  | .014 | .103 |                          |

\*Reference nickel alloy.

\*\*Reference tungsten-nickel alloy.

As shown by the test curves of Fig. 1, the yield strengths of the tungsten-titanium-nickel cathode alloys of Table A are significantly higher than those of both the reference-nickel and the reference tungsten-nickel cathode alloys throughout a high temperature range including cathode-operating temperatures in the vicinity of 1650° F. In general, as determined by these tests, the hot yield strength of the tungsten-titanium-nickel cathode alloys is about 2½ to 3 times greater than that of nickel-cathode alloy #220 and significantly higher than that of the A31 tungsten-nickel alloy. Shock tests on a production tube type (6AQ5) show a direct correlation between the shock deformation characteristics of indirectly-heated cathodes and the yield strength of the same cathode alloy at a similar temperature.

The presence of higher cobalt content in the #552 and #5514 alloys increases the yield strength at temperatures below about 1300° F. but has little or no effect at temperatures in the neighborhood of 1600° F. For this rea-

son and because of its general shortage, cobalt need not be included, or added, in amounts more than 1%. The amount of aluminum added was found not to affect the yield strength of the tungsten-titanium-nickel alloys at cathode-operating temperatures, although possibly also serving to result in precipitation hardening at lower temperatures.

The emission characteristics of oxide-coated cathodes using the nickel and tungsten-titanium-nickel alloys of Table A are shown in Figs. 2A, 2B, 3A, 3B, 4A and 4B. In these figures, each curve is identified by the respective alloy designation presented in Table A. For these emission tests, the cathodes were utilized in the standard diode structure defined in Spec. F270-52T of ASTM (American Society of Testing Materials).

The cathode sleeves were 0.45 inch, O. D. x 0.002 inch wall x 27 mm. long. The life burning conditions were an anode-cathode supply voltage ( $E_b$ ) of 100 volts, a heater voltage ( $E_f$ ) of 6.5 volts, and a load resistance ( $R_b$ ) of 1000 ohms. Anode current readings were taken at 0, 5, 25, 56, 100, 200, 350 and 500 hours, and from then every 250 hours to the end of the test. At each of these test times, the anode current was read for plate voltage of 40 volts for a number of heater voltages including the normal voltage ( $E_f=6.5$  volts) and subnormal voltages (including  $E_f=4.5$  volts). Such anode current readings plotted against time constitute the curves of Figs. 2A, 2B, 3A and 3B. The  $I_s$ FM or direct-current emission figure of merit curves of Figs. 4A, 4B are derived from these anode-current vs. heater-voltage readings as described in detail in an article of Briggs and Richard in the ASTM bulletin for January 1951. Briefly, the  $I_s$ FM value is the ratio of the  $I_b$ ,  $E_f$  coordinates at the knee of the anode current/heater voltage curve where the anode-current changes from a space charge limited condition to a temperature-limited condition (subnormal heater voltage). For comparison purposes, the emission curves for tubes having #220 nickel cathodes are also shown in Figs. 2A-4A, 4B. The corresponding curves for tubes having the Cathaloy A-31 alloy reference cathodes are not shown since they are substantially similar to those of the #220 alloy cathodes. Emission test curves

for the #54053 alloy were not obtained since this heat was essentially a duplicate of #54027.

Referring to Figs. 2A, 2B, and 4B, the indirectly-heated cathodes of alloys #552 and #5514 activated more rapidly than the #220 alloy reference cathodes. Specifically, the #552 cathodes were activated by 14 hours of life with an FM value of 14.5: the #5514 cathodes were activated by 19 hours of life with an FM value of 14.8: the reference cathodes required 22 hours of life to reach an FM value of 14.5.

After activation and until near the end of the life tests, the emission characteristics of the #552 cathodes were lower than those of the reference cathode, particularly at subnormal heater voltage. Near the end of the life tests, the emission, for normal heater voltage of the #552 cathodes, slowly rose to match or cross the falling emission of the reference cathodes (Fig. 2A). Throughout the life tests, the emission characteristics of the #5514 cathodes were consistently higher than those of

the reference cathodes. This is shown by Figs. 2A, 2B and 4B for all three methods of evaluation.

Examination of the cathodes after life testing indicated some peeling of the oxide coating of the #552 cathodes. This is attributed to the slightly higher aluminum content of the #552 cathodes and is explanatory of the difference between the emissions of the #552 and #5514 cathodes during life. The beneficial effect upon emission of the lower percentage of titanium in the #552 alloy was obscured, until late in life, by the peeling effect due to excess aluminum. The beneficial effect, both upon mechanical and emission characteristics of addition of titanium in amounts as small as 0.15% in the #552 alloy can be realized by properly limiting the concentration of any aluminum included for its activation effects.

It was determined from examination of the life-tested cathodes and by tests conducted with uncoated cathodes in special sublimation tubes that the additives tungsten and titanium in the #552 and #5514 cathodes did not contribute to formation of sublimation deposits and did not result in harmful interface-impedance.

Referring to Figs. 3A, 3B and 4A the indirectly-heated cathodes of alloy #54027 activated more slowly than the #220 reference cathodes, requiring 50 hours to reach an FM value of 15.3, whereas the reference cathodes required 32 hours to reach an FM value of 15.5. However, after the first 350 hours of testing, the emission characteristics of the #54027 cathode surpassed and remained higher than those of the #220 cathodes for the remainder of the life test period. At the end of the test period, the FM value of the #54027 cathodes was 14.8, whereas the FM value of the reference cathodes had fallen to 14.2.

It was determined by examination of the life-tested cathodes and by tests conducted with uncoated cathodes in special sublimation tubes that the additives tungsten and titanium in the #54027 cathodes did not contribute to the formation of sublimation deposits or result in harmful interface-impedance. In fact, the #54027 alloy containing the highest amount of titanium had the lowest sublimation rate of all, indicating a favorable reaction between titanium and one or more of the subliming elements, nickel, magnesium, copper and/or manganese, thereby reducing the sublimation rate of the alloy.

The tungsten-titanium-nickel cathodes have a resistance to deformation, which at cathode-operating temperatures, is at least several times that of the reference-nickel cathodes, and which also when the aluminum content, if any, is held to suitably low controlled values, have emission characteristics which are stable and equal to or better than those of the reference-nickel cathodes. Since the cathodes have nearly the same physical strength throughout the range of about 0.15% to 3% titanium, and since titanium serves both as an activating and a strengthening agent, the more exact selection of the titanium percentage may be made on the basis of its

effect on the electrical properties of the cathodes. As indicated above, for titanium percentages in the range of from about 0.4% to 3%, the emission characteristics are superior to those of the reference cathodes and for the higher percentages of this range, the sublimation rate is definitely lower than that of the reference cathodes. For good coating adherence and low interface-impedance, the tungsten-titanium-nickel cathode alloys should not contain aluminum in excess of about 0.15% or silicon in excess of about 0.04%; neither of these properties is impaired by addition of tungsten and titanium throughout the ranges herein given.

What is claimed is:

1. An indirectly-heated cathode structure characterized by high strength at cathode-operating temperatures, sustained high level of emission and low sublimation and composed of an alloy containing tungsten in the range of 1% to 5% by weight, titanium in the range of 0.05% to 3% by weight, and the remainder essentially nickel.
2. An indirectly-heated cathode structure characterized by high strength at cathode-operating temperatures, sustained high level of emission, and negligible sublimation and composed of an alloy containing 1% to 5% tungsten, 0.05% to 3% titanium; at least one of the activating agents aluminum, magnesium and silicon in the range of not more than about 0.07% magnesium, 0.15% aluminum, 0.05% silicon; and the balance essentially nickel with not more than about 0.2% iron, 0.20% manganese, 0.08% carbon, and 0.20% copper as residuals.
3. An indirectly-heated cathode structure characterized by high strength at cathode-operating temperatures, sustained high level of emission and negligible sublimation and composed of an alloy containing from about 5% tungsten, about 3% titanium, and the balance essentially nickel with not more than about 0.20% iron, 0.20% manganese, 0.08% carbon, 0.20% copper as residuals, and not more than about 0.07% magnesium, 0.15% aluminum and 0.05% silicon for cathode activation.
4. An indirectly-heated cathode structure characterized by a strength at cathode-operating temperatures of 2½ to 3 times that of unalloyed cathode nickel, and having a composition of about 4% tungsten, 0.4% titanium, .08% aluminum, 0.08% maximum carbon, 0.04% maximum magnesium, 0.04% maximum silicon, 0.10% maximum manganese, and the balance substantially nickel.

#### References Cited in the file of this patent

#### UNITED STATES PATENTS

|    |           |         |       |                |
|----|-----------|---------|-------|----------------|
| 50 | 1,899,623 | Lowry   | ----- | Feb. 28, 1933  |
|    | 2,103,267 | Mandell | ----- | Dec. 28, 1937  |
|    | 2,172,967 | De Boer | ----- | Sept. 12, 1939 |
|    | 2,323,173 | Widell  | ----- | June 9, 1943   |
|    | 2,396,977 | Widell  | ----- | Mar. 19, 1946  |
| 55 | 2,720,458 | Kates   | ----- | Oct. 11, 1955  |

UNITED STATES PATENT OFFICE  
CERTIFICATE OF CORRECTION

Patent No. 2,836,491

May 27, 1958

Ardrey M. Bounds et al.

It is hereby certified that error appears in the printed specification of the above numbered patent requiring correction and that the said Letters Patent should read as corrected below.

Column 4, line 21, for "56" read -- 50 --.

Signed and sealed this 14th day of October 1958.

(SEAL)  
Attest:

KARL H. AXLINE  
Attesting Officer

ROBERT C. WATSON  
Commissioner of Patents